

## 1

3,252,792

### CORROSION, PITTING, AND TARNISH RESISTANT STAINLESS STEEL

William A. Morgan and David E. C. King, Ottawa, Ontario, and Robert J. McClure, Bells Corners, Ontario, Canada, assignors, by direct and mesne assignments, to Her Majesty The Queen in right of Canada as represented by the Minister of Mines and Technical Surveys  
No Drawing. Filed July 6, 1964, Ser. No. 380,674  
4 Claims. (Cl. 75—126)

This invention relates to stainless steels of martensitic and ferritic grades. This application is a continuation-in-part of application Serial No. 141,006, filed September 27, 1961 (now abandoned).

Steels of the mentioned grades are frequently referred to as those of the "400 Series" and are sometimes called "plain" chromium steels. Thus, they contain chromium in excess of about 12% and substantially no nickel. Any nickel that may occasionally be used for alloying would not be present in an amount that would impart an austentic structure to the steel.

With chromium present in an amount of about or exceeding 12%, a continuous, impermeable, non-porous film of hydrous oxide forms over the surface of the steel under oxygenating (or passive) conditions. This film imparts considerable resistance to corrosion in an oxygenating medium, but breaks down in a corrosive medium whose oxygenating power is low, such as a solution containing halogens, in which case the conditions may be said to be "active." In completely active conditions, stainless steel has somewhat better overall resistance to attack than plain carbon steels but is rather more prone to pitting and grooving. Pitting takes place when active/passive cells are formed as a result of parts of the metal surface becoming exposed by film removal. Pitting is promoted in crevices in the metal surface, as well as under foreign matter such as grit, barnacles, and the like.

## 2

In severely corrosive environments, free machining types, such as 416 and 430F, have lower resistance to pitting corrosion than the corresponding unresulphurized types 410 and 430, respectively.

5 This problem of pitting corrosion in the 400 Series of stainless steels has long been recognized and additions of nickel or molybdenum have been made to such steels to improve the resistance thereof. Tarnishing or discolouration may occur as a result of any form of attack and is undesirable where an attractive surface is required, such as car trim for which 430 stainless steel is normally used.

10 It is an object of this invention to provide a chromium stainless steel having improved resistance to tarnishing, pitting corrosion and overall corrosion consistent with low cost.

15 It has been found that, when uranium is added as an alloying constituent in chromium stainless steels, substantially improved overall and pitting corrosion resistance and resistance to tarnishing is imparted to such steels. The uranium is added in an amount of 0.001-3.0% of the steel, depending on the levels of the other major elements present.

20 A large range of ferrous alloys were prepared; compositions of the main alloying elements ranging within the limits shown in Table 1.

TABLE 1

|    |                                 | Percent   |
|----|---------------------------------|-----------|
| 30 | Carbon -----                    | 0.03-0.8  |
|    | Chromium -----                  | 11.5-35   |
|    | Uranium -----                   | 0.001-2.0 |
|    | Nickel (when present) -----     | Up to 2.5 |
| 35 | Molybdenum (when present) ----- | Up to 1.0 |

Corrosion tests on steels of such compositions have been carried out using an aerated solution of 10%  $\text{FeCl}_3 \cdot 6\text{H}_2\text{O}$  in 0.05 N HCl. This solution was chosen

TABLE 2

*Pitting corrosion table showing the effect of a 4 hour exposure to acidified ferric chloride on weight loss per unit area and surface appearance*

| Structure        | Composition, percent |      |      |        |              | U/C Ratio | Weight loss, grams/sq. cm. | Surface Appearance                                    |
|------------------|----------------------|------|------|--------|--------------|-----------|----------------------------|-------------------------------------------------------|
|                  | Cr                   | Ni   | C    | U      | Other        |           |                            |                                                       |
| Ferritic.....    | 13.5                 | 0    | 0.03 | 0      | 0.63 Mo..... | 0         | 0.03380                    | Granular attack with mild pitting.                    |
| Do.....          | 13.6                 | 0    | 0.03 | 0.22   | 0.64 Mo..... | 7.34      | 0.03290                    | Granular attack only.                                 |
| Do.....          | 14.0                 |      | 0.04 | 0      |              | 0         | 0.03340                    | Deep granular attack.                                 |
| Do.....          | 14.1                 |      | 0.04 | 0.35   |              | 8.76      | 0.03200                    | Fairly deep granular attack.                          |
| Do.....          | 14.0                 |      | 0.04 | 1.89   |              | 22.25     | 0.00614                    | Surface brighter. Pinhole attack.                     |
| Do.....          | 13.8                 |      | 0.04 | 1.43   |              | 35.75     | 0.0116                     | Surface bright. Pinhole attack.                       |
| Martensitic..... | 11.8                 | 1.96 | 0.10 | 0      |              | 0         | 0.0294                     | Surface tarnished. Heavy pinhole and granular attack. |
| Do.....          | 11.7                 | 1.89 | 0.09 | 0.48   |              | 5.33      | 0.00857                    | Surface slightly tarnished.                           |
| Do.....          | 11.6                 | 1.90 | 0.09 | 1.29   |              | 14.34     | 0.00552                    | Few pinholes.                                         |
| Do.....          | 11.5                 | 1.82 | 0.11 | 1.87   |              | 17.00     | 0.00788                    | Surface bright. Some pinhole attack.                  |
| Ferritic.....    | 17.2                 |      | 0.10 | 0      |              | 0         | 0.02385                    | Very slightly tarnished with granular attack.         |
| Do.....          | 17.5                 |      | 0.10 | 0.0036 |              | 0.036     | 0.01890                    | Fairly heavy granular attack with small pits.         |
| Do.....          | 17.4                 |      | 0.10 | 0.046  |              | 0.46      | 0.01875                    | Surface somewhat tarnished with small pits.           |
| Do.....          | 17.2                 |      | 0.10 | 0.27   |              | 2.70      | 0.00921                    | Surface less tarnished with fewer small pits.         |
| Do.....          | 24.6                 |      | 0.20 | 0      |              | 0         | 0.02165                    | Surface bright with some pinholes.                    |
| Do.....          | 24.7                 |      | 0.20 | 0.042  |              | 0.21      | 0.01130                    | Surface bright with fewer pinholes.                   |

for its ability to attack the oxide film and to promote pitting. Tests have been carried out on a number of such steels in the as forged condition. Results of these tests are shown in Table 2. The microstructure of these steels therefore results from air cooling from about 1600° F., which, in chromium steels, would be equivalent to quenching from that temperature.

The improvement in corrosion resistant properties bears direct relationship to the ratio of uranium to carbon but this cannot be attributable to stabilization because of the fact that the steels had cooled quickly through the sensitization range.

Improved resistance to corrosion has also been obtained when alloys were tested in appropriate heat treated conditions.

If steels are used in operating conditions which involve the risk of sensitization the presence of uranium in sufficient quantity will also stabilize them and thereby protect them against grain boundary corrosion.

It is evident from the results quoted in Table 2 that uranium has improved the corrosion resistance, pitting resistance and tarnishing resistance, of a wide range of steels of ferritic and martensitic structure, but more particularly the martensitic grades and the type 430 ferritic steels (7 to 14 of Table 2). In the martensitic steels the addition of 0.48 to 1.87% of uranium and in the type 430 steels the addition of 0.0036 to 0.30% uranium shows a marked continuing improvement in corrosion resistance and brightness. For any particular base composition the corrosion resistance appears to vary directly as the ratio of uranium to carbon. When the base alloy contains more chromium, or more nickel, the added corrosion resistance obtained is considerably enhanced by the presence of uranium so that optimum effects are obtained with lower uranium to carbon ratios. When the base alloy contains more carbon, more uranium is

required to maintain a given uranium to carbon ratio, so that it is desirable to maintain the lowest levels of carbon permissible in the various grades. However, in view of the effect of high chromium in lowering the required optimum uranium to carbon ratio, alloys containing high carbon could be used provided they are accompanied by high chromium contents.

The concentration of the main elements Cr, C, U, and Ni and alloying elements such as Mo (where special structural modifications are required) should fall within the limits specified for the required grade and Table 1. The concentrations of Mn, Si, S and P should fall within the ranges usually associated with chromium stainless steels, including the resulphurized grades 416 and 430 F.

15 We claim:

1. A ferrous alloy of the chromium stainless steel type consisting essentially of carbon about 0.09-0.11%, chromium about 11.5-17.5%, nickel when present up to about 2.5%, uranium about .0036-2.0%, and balance iron.

2. A ferrous alloy of the chromium stainless steel type consisting essentially of carbon approximately 0.10%, chromium approximately 17%, uranium 0.0036-0.30%, and balance iron.

25 3. A ferrous alloy of the chromium stainless steel type consisting essentially of carbon approximately 0.10%, chromium approximately 14-18%, uranium 0.0036%, and balance iron.

4. A ferrous alloy of the chromium stainless steel type 30 consisting essentially of carbon approximately 0.10%, chromium 14-18%, uranium 0.001-1.0% and balance iron.

No references cited.

35 DAVID L. RECK, *Primary Examiner.*

P. WEINSTEIN, *Assistant Examiner.*